# EUROPEAN PATENT SPECIFICATION

(11) **EP 4 305 131 B1**
(45) Date of publication and mention of the grant of the patent: **11.12.2024**
(21) Application number: 22701202.8
(22) Date of filing: 14.01.2022
(51) Int. Cl.: C10M 107/34

(54) **LOW VISCOSITY FUNCTIONAL FLUID COMPOSITION**
NIEDRIGVISKOSE FUNKTIONSFLÜSSIGKEITSZUSAMMENSETZUNG
COMPOSITION DE LIQUIDE FONCTIONNELLE AVEC UNE VISCOSITÉ BASSE

(30) Priority: 12.03.2021 EP 21162202
(43) Date of publication of application: 17.01.2024
(73) Proprietor: Clariant International Ltd, 4132 Muttenz (CH)
(72) Inventor: HÖVELMANN, Felix, 84453 Mühldorf (DE); ENDRES, Andreas, 89264 Weißenhorn (DE)
(74) Representative: Clariant Produkte (Deutschland) GmbH
(86) International application number: PCT/EP2022/050757
(87) International publication number: WO 2022/189047

(56) References cited:
- WO-A2-2007/005593
- GB-A- 1 330 468

## Description

The present invention relates to a low viscosity functional fluid composition comprising a mixture of alkyl polyglycols, polyglycols and additives, the fluid being virtually free of boric acid esters of glycols or alkyl polyglycols. The fluid exhibits a low temperature kinematic viscosity of less than 900 centistokes, determined at -40°C, exhibits an equilibrium reflux boiling point (ERBP) of at least 250°C and a wet equilibrium reflux boiling point (WERBP) of at least 165°C, according to the methods described in the Federal Motor Vehicle Safety Standards (FMVSS) No 116.

The low viscosity functional fluid composition according to the present invention is useful in a variety of applications and in particular as a brake fluid, especially for new electronic or automated anti-lock brake systems which require lower viscosity fluids for satisfactory operation at low temperatures.

Functional fluid compositions based on borate esters are well known in the art. To be useful for example as DOT 4 or DOT 5.1 brake fluids, these borate ester based compositions must meet stringent physical properties and performance requirements particularly with respect to minimum dry equilibrium reflux boiling point ("ERBP"), minimum wet equilibrium reflux boiling point ("WERBP") and maximum low temperature kinematic viscosity (e.g. determined at -40°C) while maintaining adequate resistance to corrosion, stability and meeting other physical property requirements such as pH, reserve alkalinity, corrosion protection and rubber swelling.

While borate esters are advantageous to meet the DOT 4 and DOT 5.1 criteria according to Federal Motor Vehicle Safety Standards (FMVSS) No 116, especially a very high wet boiling point (wERBP), borate containing brake fluids are associated with problems. Federal Motor Vehicle Safety Standards (FMVSS)

No 116 refers to 49 CFR § 571.116 in the 10-1-2016 edition and will be referred to as FMVSS in this specification.
1. Boric acid is known to be a CMR-compound (repro tox category 1). Therefore, also its esters are suspect to similar health threat (currently classified as repro tox category 2) and, therefore of potential danger during handling/filling of the brake fluid.
2. Borate-esters of alkyl glycols are more hygroscopic compared to the sole alkyl glycols, resulting in an elevated water uptake from moisture of borate-containing brake fluids, which is undesired during storage and use.
3. The content of boron in the brake fluids is associated with a certain risk of gel formation or precipitation due to salt formation of the inorganic character of boron salts, especially upon ageing of the brake fluids As a result, particles may occur in the brake fluid and limit its performance in critical situations.

WO-00/65001 describes hydraulic fluids comprising alkoxy glycol borate esters, alkoxy glycols and corrosion inhibitors, additionally containing cyclic carboxylic acid derivatives.

WO-02/38711 describes low viscosity functional fluid compositions comprising alkoxy glycol borate esters, alkoxy glycol components and additives such as corrosion inhibitors, wherein the alkoxylation degrees of the alkoxy glycol borate esters and the alkoxy glycols are restricted to a certain narrow pattern.

US-4371448A teaches a hydraulic fluid which formally fulfils the specification DOT 5. This hydraulic fluid essentially consists of (A) about 20 to 40% by weight of at least one boric acid ester obtained from orthoboric acid, diethylene glycol and an ethylene glycol monoalkyl ether; (B) 30 to 60% by weight of at least one ethylene glycol monoalkyl ether; (C) 10 to 40% by weight of at least one bis-(ethylene glycol monoalkyl ether)-formal; (D) 0.1 to 5% by weight of at least one alkylamine; and (E) 0.05 to 5% by weight of at least one stabilizer and/or inhibitor; the percentages by weight in each case being relative to the total weight of the fluid.

EP-0750033A1 teaches a hydraulic fluid composition, especially a brake fluid composition, based on a boric ester of a glycol ether and comprising a corrosion-inhibiting system which includes: (1) at least one constituent (A) chosen from fatty amines or the salts of one or more carboxylic acids with the said amines, and (2) at least one constituent (B) chosen from the products resulting from the reaction of one or more carboxylic fatty acids with a polyoxyalkylene glycol, or from the transesterification reaction of one or more esters of carboxylic fatty acids with a polyoxyalkylene glycol.

EP-0617116A1 teaches a hydraulic fluid composition having a high boiling point, in particular a high equilibrium reflux boiling point and a low viscosity. The composition contains, as additive, at least one ether amine having a molecular weight between 120 and 300 and having the formula in which
- R₃: is linear or branched radical having at least one ether functional group and no alcohol functional group,
- R: is a methyl radical or a hydrogen atom,
- p: is an integer from 1 to 3 and
- q: is an integer from 0 to 2.

WO-2012/003117A1 discloses a functional fluid composition comprising
(i) an alkoxy glycol mixture in an amount of about 38% to 47% by weight of the functional fluid composition, where the alkoxy glycol mixture is comprised alkoxy glycols having the formula with repeat unit: wherein
   each of R₁ , R₂, R₃, R₄, R₅ is either hydrogen (H) or an alkyl group containing 1 to 8 or more carbon atoms or mixtures thereof, wherein said mixture has a first alkoxy glycol component in an amount of about 36% to about 73% by weight of said mixture where n = 3, a second alkoxy glycol component from 17% to about 43% by weight of said mixture where n = 4, and a third alkoxy glycol component in an amount from about 2% to about 10% by weight of said mixture where n is greater than or equal to 5 and
(ii) a glycol borate ester in an amount of about 53% to 62% by weight of the functional fluid composition.

EP-A-0129240 teaches hydraulic fluids with a boron content of from 0 to 1 % by weight, and consisting essentially of
a) 2 - 40% by weight, of an alkylene glycol of general formula (I):

   HO - (RₐO)ₓ - H (I)

   wherein
   - Rₐ: is an alkylene radical having from 2 to 3 carbon atoms, and
   - x: is an integer between 1 and 3;
b) 15 - 65% by weight, referred to the total weight of the fluid, of an alkylene glycol mono alkylether of general formula (II);

   R - (RₐO)ₓ - OH (II)

   wherein
   - Rₐ and x: have the above indicated meanings, and
   - R: is a C₁ -C₄ alkyl;
c) 15 - 55% by weight, referred to the total weight of the fluid, of at least one poly alkylene glycol mono alkylether of general formula (III)

   R - (OCHR'CH₂)ₙ - OH (III)

   wherein
   - R: is a C₁ -C₄ alkyl;
   - R': is H or CH₃ and
   - n: is an integer whereby the molecular weight of the compound will be between 208 and 1000;
d) 0 - 54% by weight, referred to the total weight of the fluid, of the reaction product of H₃ BO₃ with the alkylene glycols of formula (I), in a molar ratio of 1 : 1.5 - 3;
e) 0 - 10% by weight, referred to the total weight of the fluid, of at least one inhibitor.

DE-3627432 teaches a brake fluid based on glycols and glycol ethers, consisting essentially of
A) 30 to 80% by weight, based on the total weight of the brake fluid, of a glycol component, consisting of
   a) 0 to 80% by weight diethylene glycol and / or dipropylene glycol and
   b) 20 to 100% by weight of triethylene glycol, tripropylene glycol, tetraethylene glycol and / or tetrapropylene glycol, percent by weight based on the mixture of these glycols,
B) 20 to 70% by weight, based on the total weight of the brake fluid, of a glycol ether component, consisting of
   a) 10 to 100% by weight-% of at least one glycol dialkyl ether of the following formula R- (OAlk₁) x-OR1, in which R and R1 are an alkyl group with 1 to 4 C atoms, Alk₁ is the ethylene or a propylene group and x is an integer from 3 to 6, and
   b) 0 to 90 wt. -% of at least one glycol monoalkyl ether of the following formula R2- (OAlk₂) y-OH, in which R2 is an alkyl group with 1 to 4 carbon atoms, Alk₂ is the ethylene or a propylene group and y is an integer from 2 to 4, percent by weight based on the mixture of these glycol ethers, and
C) 0 to 5% by weight, based on the total weight of the brake fluid, of at least one inhibitor for fluids based on glycol and glycol ethers, with the proviso that at least 14% by weight in the brake fluid of the glycol component b) are contained, weight percent based on the total weight of the brake fluid.

GB-1330468 describes brake fluid compositions containing orthoesters of the formulae A and B in combination with polyoxyalkyleneglycol esters of dicarboxylic acids and/or alkyl esters of glycols or polyglycols

Such compounds were applied in 10 wt.-% in base fluid, consisting of mainly conventional esters, such as propionates and nylonates and minor amounts of alkyl glycols. The addition of 10% of various ortho esters resulted in a less pronounced reduction of boiling point in the presence of 1 wt.-% water (minus 69°C and less, compared to -100°C reduction in the absence of ortho esters). Yet, the impact on water uptake and in the standardized WERBP test according to FMVSS no. 116 was not known. In addition, the viscosity of the functional fluids according to Castrol GB-1330468 was rather high with around 1700 cSt at - 40°C.

There is a strong demand for improved high performance hydraulic fluid compositions and brake fluids having low temperature viscosity at -40°C while meeting or exceeding at the same time the minimum ERBP and especially the WERBP temperature requirements, as fulfilled by the hydraulic fluid compositions and brake fluids commonly used.

Examples of borate-free brake fluids are described in the literature
1.) DOT3/class 3 fluids, which are in general of a lower ERBP, lower wERBP and higher viscosity at -40°C), according to FMVSS.
2.) GB-1330468 (Castrol) discloses borate-free brake fluids, containing ortho esters in combinations with poly oxyalkylene glycol ether-ester of dicarboxylic acids and/or alkyl ester of glycols or polyglycols and minor amounts of alkylglycols. Such combinations suffer from elevated viscosity at -40°C and the WERBP was not investigated.
3.) DE-3627432C2 (Hoechst) and US-2006/0264337 (BASF) disclose diethylene/triethylene glycol and dipropylene glycol based brake fluids, fulfilling just the minimum requirement of DOT 4 and ISO 4925 class 4 norm.
4.) WO-2007/005593A2 (DOW) describes compositions of brake fluids containing 0-10 wt.-% of borate ester and the use of larger quantities of butoxy-glycols, mainly butoxy-triglycol.
5.) EP-0129240A1 (Montedison S.p.A.) discloses borate-free brake fluid formulations consisting of min. 30 wt.-% diethylene glycol or higher glycols but suffering from elevated viscosity at -40°C.

These developments allow for high ERBP but suffer from a still too high viscosity at -40°C and from a low WERBP. The problem to be solved by the instant invention is to provide a hydraulic fluid having the properties mentioned below and being essentially or entirely borate free.

| | GB-1330468 (Castrol) mixture 1 | WO-2007/005593 (DOW) | US-2006/0264337 (BASF) "BF1" | DE-3627432 (Examples) | EP-0129240 Example 1 | Target of the present invention |
|---|---|---|---|---|---|---|
| ERBP [°C] | 310 | 270 | 251 | 237-277 | 250 | min. 250 |
| WERBP [°C] | Not studied | 145 | 159 | 144-158 | 161 | min. 165 |
| Viscosity at -40°C [cSt] | 1694 | 859 | 1393 | 1000-1450 | 1276 | max. 900 |

Yet, a borate-free composition, fulfilling these criteria is not known.

According to the present invention, a functional fluid composition being essentially free from borates has been found which exhibits superior values of ERBP and of WERBP and for low temperature kinematic viscosity, while maintaining excellent resistance to corrosion, high stability and meeting other physical property requirements such as pH, reserve alkalinity and rubber swell. Especially very high WERBP values are achieved by using ortho esters as a replacement for borate esters.

In a first aspect, this invention relates to a functional fluid, comprising
(A) from 8 to 80% by weight, based on the total composition, of one or more ortho-ester according to formula (I) wherein
   - R₁, R₂, R₃: are independently selected from H or C₁ to C₈ alkyl groups, preferably methyl or butyl,
   - R₄: means H or C₁ to C₈ alkyl, preferably H or methyl,
   - a, b, c: are independently numbers from 0 to 6, preferably 3 or 4,
   with the proviso that a+b+c is at least 1,
(B) from 10 to 87% by weight, based on the total composition, of one or more alkoxy glycol according to formula (II)

   R₅ - O - (CH₂ - CH₂ - O)ₘ - H (II)

   wherein
   - R₅: is a C₁ to C₈ alkyl residue, preferably methyl or butyl,
   - m: is a number from 2 to 6, preferably 3 or 4,
(C) from 0 to 20, preferably 8 - 18 wt.-% of at least one compound according to formula (III)

   H -O- (CH₂ - CH₂ - O)ₖ - H (III)

   wherein k is a number of 2 or higher, with the proviso that in at least 80 wt.-% of all compounds according to formula (III) k is 2 or 3,
(D) at least one additive, selected from the group consisting of corrosion inhibitor, alkalinity agents, aging protection agents, defoamers and lubricants,

the fluid comprising at most 3 wt.-% of an ester between boric acid and a glycol or polyglycol compound, and
with the proviso that the combined amount of component (A) and component (B) adds up to at least 70 % of the total fluid weight.

In a second aspect, this invention provides the use of the functional fluid of the first aspect as a brake fluid for vehicular brakes.

In a third aspect, this invention provides for a method of operating a vehicular brake that transmits braking force through a hydraulic system, the method comprising filling the hydraulic system with a functional fluid according to the first aspect.

The functional fluid will be referred to as fluid in the following.

### Component (A) - Orthoester

The orthoester used as component (A) corresponds to one or more components according to formula (I).

In formula (I), R1, R2, R3 are independently selected from H or C₁ to C₈ alkyl groups preferably from H or C₁ to C₄ alkyl groups. In a preferred embodiment, R1, R2, R3 are independently selected from methyl or butyl. In a more preferred embodiment, R1, R2, R3 mean methyl. In a preferred embodiment, only one out of R1, R2, R3 takes the meaning of H. In another preferred embodiment, the amount of orthoester according to formula (I) wherein at least one of R1, R2, R3 takes the meaning H is less than 30 wt.-%, more preferably less than 15 wt.-%, particularly less than 10 wt.-%, on a basis of 100 wt.-% being the total amount of all orthoester according to formula (I). In a preferred embodiment, the orthoester used as component (A) corresponds to two or more components according to formula (I).

It is preferred, that the two or more orthoesters of formula (I) differ in one out of R1, R2, R3. This may mean e.g. that one out of R1, R2, R3 is methyl in one of the orthoesters, and one out of R1, R2, R3 is butyl in the other of the orthoesters.

In formula (I), R4 means H or C₁ to C₈ alkyl. In a preferred embodiment, R4 means H or methyl.

In formula (I), a, b, c are independently numbers from 0 to 6, with the proviso that a+b+c is at least 1, i.e. not all of a, b, c may equal zero. In a preferred embodiment, a, b, c are independently 3 or 4. In another preferred embodiment, a+b+c is at least 3, more preferably at least 6. In a preferred embodiment, the orthoester used as component (A) corresponds to two or more components according to formula (I). It is preferred, that the two or more orthoesters of formula (I) differ in one out of a, b, c., meaning that a, b, c are not all the same in the two or more orthoesters. For example, one out of a, b, c may be 3 in one of the orthoesters, and one out of a, b, c may be 4 in the other of the orthoesters.

The orthoester should be clear, homogeneous, and substantially free of salt or suspended components, e.g. such as residues of insoluble catalysts, to render a clear, homogenous functional fluid.

In a further preferred embodiment, the orthoester used as component (A) is not a single compound, but a mixture of at least two orthoesters according to formula (I) and (Ia). This means that in one embodiment, the fluid according to the first aspect not only comprises an orthoester according to formula (I), but in addition a bridged orthoester according to formula (Ia) wherein R1, R2, R4, a and b have the same meaning as provided for formula (I), and d is a number from 0 to 6, preferably 2 or 3.

In formula (Ia), R1, R2 are independently selected from H or C₁ to C₈ alkyl groups preferably from H or C₁ to C₄ alkyl groups. In a preferred embodiment, R1, R2 are independently selected from methyl or butyl. In a more preferred embodiment, R1, R2 mean methyl. In a preferred embodiment, only one out of R1, R2 takes the meaning of H. In another preferred embodiment, the amount of orthoester according to formula (Ia) wherein at least one of R1, R2 takes the meaning H is less than 30 wt.-%, more preferably less than 15 wt.-%, particularly less than 10 wt.-%, on a basis of 100 wt.-% being the total amount of all orthoester according to formula (Ia). In a preferred embodiment, the orthoester used as component (A) corresponds to two or more components according to formula (Ia).

It is preferred, that the two or more orthoesters of formula (Ia) differ in one out of R1, R2. This may mean e.g. that one out of R1, R2 is methyl in one of the orthoesters, and one out of R1, R2 is butyl in the other of the orthoesters.

In formula (Ia), R4 means H or C₁ to C₈ alkyl. In a preferred embodiment, R4 means H or methyl.

In formula (Ia), a, b are independently numbers from 0 to 6, with the proviso that a+b is at least 1, i.e. not all of a, b, c may equal zero. In a preferred embodiment, a, b are independently 3 or 4. In another preferred embodiment, a+b is at least 3, more preferably at least 6. In a preferred embodiment, the orthoester used as component (A) corresponds to two or more components according to formula (Ia). It is preferred, that the two or more orthoesters of formula (Ia) differ in one out of a, b, meaning that a, b are not all the same in the two or more orthoesters according to formula (Ia). For example, one out of a, b may be 3 in one of the orthoesters, and one out of a, b may be 4 in the other of the orthoesters.

If a bridged orthoester according to formula (Ia) is present, its amount is preferably at most 30 wt.-%, more preferably less than 15 wt.-%, particularly less than 10 wt.-%, on a basis of 100 wt.-% being the total amount of all orthoester according to formula (I). For the purposes of this invention, the bridged orthoester according to formula (Ia) is to be regarded as part of component A). The amount of orthoester according to formula (Ia) is to be counted within the amount of component (A).

The bridging of orthoester by polyalkylene glycols has the technical effect of increasing the viscosity of the orthoester component, and therefore increasing the viscosity of the fluid of the first aspect. A larger proportion of bridged orthoesters of the formula (Ia) provides a higher viscosity of the fluid.

Orthoesters according to formula (I) and (Ia) can be synthesized according to procedures known in the art from alkyl glycols and commercially available alkyl ortho esters, according to

Useful alkyl ortho esters are selected from R4 being a H or C₁- to C₈-akyl residues and Rx being C₁- bis C₆-alkyl residues.

The alkyl glycol reactant of formula (IV) comprises species of ethoxylation degree of from y = 1 to y = 6, preferably of from y = 2 to y = 4, more preferably of y = 3 to y = 4. It is to be understood that the alkyl glycol reactant may be a single species, or a mixture of different species with regards to their ethoxylation degree y and/or to radicals R1, R2 and R3.

Radicals R1, R2 and R3 are preferably C₁- to C₄-alkyl groups and may be methyl, ethyl, n-propyl, isopropyl, n-butyl, isobutyl, sec-butyl, tert-butyl, preferably n-butyl or methyl.

Examples of useful alkoxy glycols as starting material for component (A) of the present invention wherein R1, R2 or R3 is not H include methyldiglycol, methyltriglycol, methyltetraglycol, methylpentaglycol, methylhexaglycol, ethyldiglycol, ethyltriglycol, ethyltetraglycol, ethylpentaglycol, ethylhexaglycol, n-propyl-diglycol, n-propyltriglycol, n-propyltetraglycol, n-propylpentaglycol, n-propylhexaglycol, n-butyldiglycol, n-butyltriglycol, n-butyltetraglycol, n-butylpentaglycol, n-butylhexaglycol, n-pentyldiglycol, n-pentyltriglycol, n-pentyltetraglycol, n-pentylpentaglycol, n-pentyl-hexaglycol, n-hexyldiglycol, n-hexyltriglycol, n-hexyltetraglycol, n-hexylpentaglycol, n-hexylhexaglycol, 2-ethylhexyldiglycol, 2-ethylhexyltriglycol, 2-ethylhexyltetraglycol, 2-ethylhexylpentaglycol, 2-ethylhexylhexaglycol and mixtures thereof. For the avoidance of doubt, "glycol" herein always means "ethylene glycol".

Example for useful glycols as starting material for component (A) of the present invention wherein R1, R2 or R3 is H include preferably diethyleneglycol, triethyleneglycol and tetraethylene glycol and mixtures thereof.

In general, hydraulic fluids require the presence of agents providing reserve alkalinity. Such agents are e.g. amines. The required amount of the amine component is dependent on the required reserve alkalinity and the required pH value of the final functional fluids. Both reserve alkalinity and pH contribute to corrosion inhibition.

Borate-ester containing brake fluids require higher amounts of amine, usually above 1 wt.-%, in order to maintain a pH value in the range of 7.0 to 11.5, even upon hydrolysis of borate esters into the triprotic boric acid and the corresponding glycols.

In contrast, ortho-ester based brake fluids require reduced amounts of amine. Hydrolysis of ortho esters results in the formation of two equivalents of the corresponding alcohols, and one equivalent of the corresponding ester. As an example, the hydrolysis of an orthoacetate to the corresponding alcohol, and the acetic acid ester, follows this reaction path:

In a subsequent hydrolysis step, the ester (e.g. acetic acid ester) may be cleaved into the corresponding alcohol and one equivalent of the mono protic acid, e.g. acetic acid. The requirement of orthoester based fluids for reserve alkalinity is therefore reduced when compared to borate based fluids.

### Component (B) - Alkylglycol ether

Component (B) of the functional fluid composition according to general formula (II) comprises species of ethoxylation degree of from m = 2 to m = 6, preferably of from m = 2 to m = 4, more preferably of m = 3 to m = 4. Component (B) may be a single species or a mixture of different species with regards to the ethoxylation degree, and/or to R5. R5 is a C₁- to C₈-alkyl group and may be methyl, ethyl, n-propyl, isopropyl, n-butyl, isobutyl, sec-butyl, tert-butyl, n-pentyl, n-hexyl, n-heptyl, n-octyl and 2-ethylhexyl, ethyl. More preferably, R5 is ethyl, n-butyl or methyl, most preferably n-butyl or methyl.

Examples of useful alkoxy glycols for component (B) of the present invention include methyldiglycol, methyltriglycol, methyltetraglycol, methylpentaglycol, methylhexaglycol, ethyldiglycol, ethyltriglycol, ethyltetraglycol, ethylpentaglycol, ethylhexaglycol, n-propyl-diglycol, n-propyltriglycol, n-propyltetraglycol, n-propylpentaglycol, n-propylhexaglycol, n-butyldiglycol, n-butyltriglycol, n-butyltetraglycol, n-butylpentaglycol, n-butylhexaglycol, n-pentyldiglycol, n-pentyltriglycol, n-pentyltetraglycol, n-pentylpentaglycol, n-pentyl-hexaglycol, n-hexyldiglycol, n-hexyltriglycol, n-hexyltetraglycol, n-hexylpentaglycol, n-hexylhexaglycol, 2-ethylhexyldiglycol, 2-ethylhexyltriglycol, 2-ethylhexyltetraglycol, 2-ethylhexylpentaglycol, 2-ethylhexylhexaglycol and mixtures thereof. For the avoidance of doubt, "glycol" always means "ethylene glycol". From the list above, methyltriglycol, methyltetraglycol, methylpentaglycol, ethyldiglycol, ethyltriglycol, ethyltetraglycol, n-butyldiglycol, n-butyltriglycol, n-butyltetraglycol, n-butylpentaglycol, are preferred for component (B).

In a preferred embodiment, component (B) comprises a mixture of alkoxy glycols of general formula (II) comprising solely or predominantly species with m = 3 and/or 4. Predominantly shall mean that at least 60% by weight, more preferably at least 75% by weight, most preferably at least 90% by weight, of component (B) comprises species with m = 3 and/or 4. In the last case, alkoxy glycol species with m being lower than 3, e.g. with m = 2, and/or with m being higher than 4, e.g. with m = 5 and/or m = 6, may be present in minor amounts, preferably less than 10% by weight, more preferably less than 8% by weight and even more preferably less than 5% by weight. Percentages of species of component (B) are given in wt.-% with the total amount of component (B) being 100 wt.-%.

In a preferred embodiment, the proportion of component (B) is 40 - 80 wt.-% of the total fluid weight.

### Component (C) - Ethylene glycol oligomer

Component (C) is a polyethylene glycol according to formula (III). In formula (III), k is a number of 2, or higher. It is preferred, that k is a number from 2 - 4. More preferably, k is 2 or 3. In one preferred embodiment, component (C) is a mixture of compounds according to formula (III) wherein k is 2 or 3.

If component (C) is present, it is required that in at least 80 wt.-% of all compounds according to formula (III) k is 2 or 3, the wt.-% being relative to the total weight of all compounds according to formula (III). This means that compounds according to formula (III) wherein k is 2 or 3 make up to 18 wt.-%, preferably 3 to 15 wt.-% of the fluid, the total fluid weight being 100 wt.-%.

The total amount of component (C) in the fluid is from 0 to 20 wt.-%, preferably 4-18 wt.-% of the weight of the fluid, i.e. the total weight of the fluid being 100 wt.-%. In one other preferred embodiment, component (C) is absent, i.e. the amount is 0%. In one other preferred embodiment, the amount of species of formula (III) wherein k = 2 is 2 - 10wt.-%. In one other preferred embodiment, the amount of species of formula (III) wherein k = 3 is 2 - 10 wt.-%. In one other preferred embodiment, the total amount of species according to formula (III) wherein k is 4 or higher than 4 is at most 10 wt.-%, more preferably at most 6 wt.-%. Said weight percentages provided for species according to formula (III) are provided as weight percentages of the fluid, i.e. the total weight of the fluid is 100 wt.-%. They are not provided as weight percentages of the total weight of component (C).

### Component (D) - Additives

Component (D) is an additive that is required to impart particular properties to the functional fluid for performing on specifications to be fulfilled for brake fluids according to the current norms and standards FMVSS, SAE J 1703 and ISO 4925. The total amount of all components (D) in the fluid is from 0.2 to 6 wt.-%, preferably from 0.5 to 5 wt.-%.

Component (D) comprises one or more additives selected from the group consisting of corrosion inhibitors, amines as reserve alkalinity agents, stabilizing antioxidants, defoamers, lubricants and dyes.

Component (D) may comprise an amine or mixtures of amines as alkalinity agent. Amines are preferably alkyl or cycloalkyl amines, alkanol amines, alkyl amine ethoxylates and their mixtures. Preferred alkyl amines are mono- and di-(C₄- to C₂₀-alkyl)amines. Examples of suitable alkyl or cycloalkyl amines are n-butylamine, n-hexylamine, n-octylamine, 2-ethylhexylamine, isononylamine, n-decylamine, n-dodecylamine, oleylamine, d-n-propylamine, di-isopropylamine, din-butylamine, tri-n-butylamine, di-n-amylamine, cyclohexylamine, and salts of such amines. Examples of suitable alkanolamines are mono-, di- and trimethanolamine, mono-, di- and triethanolamine, mono-, di- and tri-n-propanolamine and mono-, di- and tri-isopropanolamine. Examples of suitable alkyl amine ethoxylates are such linear, cyclic or branched alkylamine ethoxylates carrying 1.5 to 5 EO moieties and an alkyl chain having 4 to 18 carbon atoms.

Component (D) of the present functional fluid composition may comprise, besides the Amine, at least one additive with corrosion inhibition action, although the alkylamine ethoxylates exhibit corrosion inhibition properties themselves. Suitable customary additives with corrosion inhibition properties include fatty acids such as lauric, palmitic, stearic or oleic acid; esters of phosphorus or phosphoric acid with aliphatic alcohols or aliphatic alcohol ethoxylates; such as ethyl phosphate, dimethyl phosphate, isopropyl phosphate, n-butyl phosphate, 2-ethylhexyl phosphate, triphenyl phosphite and diisopropyl phosphite; heterocyclic nitrogen containing organic compounds such as benzotriazole, tolyltriazole, 1,2,4-triazole, benzoimidazole, purine, adenine and derivatives of such heterocyclic organic compounds. Of course, mixtures of the above additives with corrosion inhibition action can be used.

Defoamers may be selected from groups of oil based defoamers, such as natural oils, glycerides, waxes, powdered silica, alkoxylates such es EO/PO block copolymers, silicone based defoamers, preferably modified polyether or silicone derivatives and mixtures thereof.

The fluid may include from 0 to 5% by weight, based on the total weight of the fluid, of a lubricant. Suitable lubricants are for example, propylene oxide containing alkylene oxide polymers that are optionally substituted with a C₁ to C₄ alkyl group, triglycerides, castor oil, ricinoleic acid, and ethoxylates of castor oil or ricinoleic acid and mixtures thereof. In a preferred embodiment, the lubricants are homopolymers of propylene oxide, copolymers of propylene oxide with ethylene oxide and/or butylene oxide, mono C₁ to C₄ alkyl substituted homopolymers of propylene oxide, mono C₁ to C₄ alkyl substituted copolymers of propylene oxide with ethylene oxide and/or butylene oxide, triglycerides, castor oil, ricinoleic acid, and ethoxylates of castor oil or ricinoleic acid and mixtures thereof. In case of such ethoxylates, 1 to 50 ethoxy units are preferred. In another preferred embodiment, the propylene oxide containing alkylene oxide polymers that are optionally substituted with a C₁ to C₄ alkyl group have a number average molecular weight in the range of 150 to 3000 g/mol.

Suitable age protecting agents or antioxidants are phenolic stabilizers like Bisphenols (e,g. Bisphenol A or Bisphenol M), butyl hydroxytoluene, methoxy phenols, butylated hydroxy anisole, hydroquinone derivatives; sterically hindered amines such as benzylated, alkylated or styrenated diphenylamine, styrenated phenylamine, substituted piperidine derivatives, phenothiazine derivatives or quinoline derivatives and mixtures thereof. In general, any literature known glycol stabilizing or age protecting agents could be used herein.

In one preferred embodiment, the % values (A) - (D) add up to 100% by weight.

The total content of the fluid in boric acid esters is at most 3 wt.-%, preferably less than 0.3 wt.-%. Most preferably, the fluid is free of boric acid esters.

In a preferred embodiment, the combined amount of components (A) and (B) adds up to at least 70% of the fluid weight.

The functional fluid composition of the present invention exhibits superior behavior in ERBP and WERBP temperature and simultaneously in low temperature viscosity performance. It exhibits an ERBP of at least 250°C, more preferably of at least 260°C and a WERBP of at least 165°C, more preferably at least 170°C. The functional fluid composition of the present invention exhibits a low temperature kinematic viscosity of less than 900 centistokes ("cSt") (= mm²/s), more preferably of less than 750 cSt, each determined at a temperature of -40°C. All analytical methods are described in FMVSS to which reference is made. For the purpose of this specification, ERBP and WERBP are to be determined according to FMVSS no 116.

The low viscosity functional fluid composition of the present invention is especially useful as a brake fluid, for example for vehicles such as passenger cars and trucks, especially for new electronic or automated anti-lock brake systems which require lower viscosity fluids for satisfactory operation at low temperatures.

Besides its superior behavior in ERBP and WERBP temperature and its low temperature viscosity performance, the functional fluid composition of the present invention exhibits a good corrosion protection, a good water compatibility, a mild pH value, a good stability with regard to low and high temperatures, a good oxidation stability, a good chemical stability, a good behavior towards rubber and elastomers, a good lubrication performance and good foaming behavior.

### Examples for orthoesters - Synthesis

### OE-A (MTG-Ortho acetate) Trimethylorthoacetate + Methyltriglycol

A mixture of 160.3 g (1.33 mol) trimethyl orthoacetate and 420 mL (2.66 mol) methyl triglycol is placed under nitrogen in a 1 liter four-necked flask equipped with a stirrer and a distillation attachment including a Vigreux column and heated to 165°C within 40 min. After the constant reaction temperature had been reached, a first portion of methanol was distilled off over the course of 60 minutes. The reaction temperature was increased to 185°C and held for a further 45 minutes, a total of about 83% (71 g, 2.22 mol) of the theoretical amount of methanol being distilled off. Thereafter, a further 211 ml (1.34 mol) of methyl triglycol were metered in at constant heating power, and after one hour the reaction temperature was increased to 225°C and held for one hour, further methanol being distilled off. A further 50 ml (0.32 mol) of methyl triglycol were then metered in at constant heating power, and 1.9 g of benzoic acid were added. After 3 hours, a further 0.9 g and finally another 0.4 g of benzoic acid were added after a further hour. Finally, the mixture was stirred at a reaction temperature of 235°C for a further 2 h. A total of 140 ml / 110.6 g of methanol (3.45 mol) were distilled off, which corresponds to a conversion of 86.3%. A similar conversion rate was observed by ¹H-NMR analysis.

### OE-B (MTG/MTeG-Ortho acetate) Triethylorthacetate + Methyltriglykol (MTG) and Methyltetraglykol (MTeG)

In analogy to the synthesis procedure of OE-A, Triethylorthoacetate (2.0 mol) was reacted with MTG (4.72 mol) and MTeG (1.61 mol), resulting in the corresponding product with 91% conversion according to 1H-NMR.

### OE-C (MTeG/MTG-Orthoformate) Trimethylorthoformiate + Methyltri- and methyltetraglykol

In analogy to the synthesis procedure of OE-A, Trimethylorthoformiate (2.5 mol) was reacted with MTG (6.04 mol) and MTeG (2.01 mol), resulting in the corresponding product with 93% conversion of the starting orthoformiate according to 1H-NMR.

### OE-D (MTG-Orthoformiate)

In analogy to the synthesis procedure of OE-A, Trimethylorthoformiate (2.0 mol) was reacted with MTG (7.0 mol), resulting in the corresponding product with 93% conversion of the starting orthoformiate according to 1H-NMR.

### OE-E (MTG/TEGBE-Ortho acetate)

In analogy to the synthesis procedure of OE-A, Trimethyl ortho acetate (1.8 mol) was reacted with a mixture of 70% triethyleneglycolmonobutylether and 30% tetraethyleneglycolmonobutylether (combined 6.3 mol), resulting in the corresponding product with 88% conversion according to NMR.

### OE-F (MTG/Di-Triglycol-Ortho acetate)

In analogy to the synthesis procedure of OE-A, Trimethyl ortho acetate (1.8 mol) was reacted with a mixture of 95 wt.-% triethyleneglycolmonomethylether, 2.5 wt.-% diethyleneglycol and 2.5 wt.-% triethyleneglycol (combined 5.6 mol), using phosphoric acid as a catalyst, resulting in the corresponding product with 90% conversion according to NMR.

Table with physical-chemical data (viscosity, boiling point, stability at repeated boiling, even in presence of amine).

| | | Conversion¹ | ERBP | Viscosity at -40°C | Δ (ERBP) |
|---|---|---|---|---|---|
| | | | [°C]² | [mm²/s]³ | [°C]⁴ |
| MTG-Ortho acetate | OE-A | 86% | 259 | 783 | -5 |
| MTeG/MTG-Ortho acetate | OE-B | 80% | 263 | 1292 | -3 |
| MTeG/MTG-Ortho formiate | OE-C | 81% | 267 | 1488 | -1 |
| MTG-Ortho formiate | OE-D | 93% | 264 | 588 | -3 |
| MTG/TEGBE-Ortho acetate | OE-E | 84% | 266 | 1097 | -6 |
| MTG/Di/Triglycol Orthoacetate | OE-F | 90% | 259 | 1208 | -6 |

| | | | | | |
|---|---|---|---|---|---|
| ¹ Conversion of starting ortho ester to alkyl glycol ortho ester, determined by ¹H-NMR. ² Equilibrium reflux boiling point of the corresponding ortho ester synthesis product according to the procedure described in FMVSS no 116 ³ Viscosity of the of the corresponding ortho ester synthesis product according to ASTM D 7042 ⁴ Thermal stability of the ortho ester, calculated as: (ERBP at the fourth time of determination of the same sample) - (initial ERBP). | | | | | |

### Examples for functional fluid formulations

Table 1 shows functional fluid compositions and their performance. Percentages are wt.-% with respect to the total fluid weight, unless otherwise noted.

## Claims

1. A functional fluid, comprising
(A) from 8 to 80% by weight, based on the total composition, of one or more ortho-ester according to formula (I) wherein
R1, R2, R3 are independently selected from H or C₁ to C₈ alkyl groups,
R4 means H or C₁ to C₈ alkyl,
a, b, c are independently numbers from 0 to 6,
with the proviso that a+b+c is at least 1,
(B) from 10 to 87% by weight, based on the total composition, of one or more alkoxy glycol according to formula (II)
R₅ - O - (CH₂ - CH₂ - O)ₘ - H (II)
wherein
R₅ is a C₁ to C₈ alkyl residue,
m is a number from 2 to 6,
(C) from 0 to 20 wt.-% of at least one compound according to formula (III)
H -O- (CH₂ - CH₂ - O)ₖ - H (III)
wherein k is a number of 2 or higher, with the proviso that in at least 80 wt.-% of all compounds according to formula (III) k is 2 or 3,
(D) at least one additive, selected from the group consisting of corrosion inhibitor, alkalinity agents, aging protection agents, defoamers and lubricants,
the fluid comprising at most 3 wt.-% of an ester between boric acid and a glycol or polyglycol compound, and
with the proviso that the combined amount of component (A) and component (B) adds up to at least 70 % of the total fluid weight.

2. Fluid according to claim 1, wherein the components (A) to (D) add up to 100 wt.-%.

3. Fluid according to claim 1 or 2, wherein R1, R2, R3 are independently selected from H or C₁ to C₄ alkyl groups.

4. Fluid according to one or more of claims 1 - 3, wherein R1, R2, R3 are independently selected from methyl and butyl groups.

5. Fluid according to one or more of claims 1 - 4, wherein R4 is H or C₁ to C₄ alkyl.

6. Fluid according to one or more of claims 1 - 5, wherein R4 is H or methyl.

7. Fluid according to one or more of claims 1 - 6, wherein a+b+c is at least 3, more preferably at least 6.

8. Fluid according to one or more of claims 1 - 6, wherein a, b, c are independently 3 or 4.

9. Fluid according to one or more of claims 1 - 8, wherein component (A) is a mixture of at least two compounds according to formula (I) that differ in one out of R1, R2, R3 or in one out of a, b, c.

10. Fluid according to one or more of claims 1 - 9, wherein in at least 60 wt.-% of all compounds according to formula (II) m is 3 or 4.

11. Fluid according to one or more of claims 1 - 9, wherein component (C) is present in an amount of 4 to 18 wt.-%.

12. Fluid according to one or more of claims 1 - 11, wherein in at most 10 wt.-% of all compounds according to formula (II) m is 5 or higher.

13. Fluid according to one or more of claims 1 - 12, wherein the fluid contains at most 10 wt.-% of compounds according to formula (III) wherein k is 4 or higher, the wt.-% being relative to the total weight component C.

14. Fluid according to one or more of claims 1 - 13, wherein component (D) is present in an amount of 0.2 to 6 wt.-%, preferably 0.4 to 4.5 wt.-%.

15. Fluid according to one or more of claims 1 - 14, wherein the corrosion inhibitor is selected from the group consisting of C₈ to C₂₂ fatty acids, esters of phosphorus or phosphoric acid with C₁ to C₁₈ aliphatic alcohols, phosphites having at least one C₁ to C₁₂ hydrocarbon residue; heterocyclic organic compounds having at least one nitrogen atom as heteroatom, and mixtures thereof.

16. Fluid according to one or more of claims 1 - 15, wherein the alkalinity agent is selected from the group consisting of alkyl or cycloalkyl amines, alkanol amines, alkyl amine ethoxylates and their mixtures.

17. Fluid according to one or more of claims 1 - 16, wherein the age protecting agent is selected from the group consisting of substituted phenols, sterically hindered amines and mixtures thereof.

18. Fluid according to one or more of claims 1 - 17, wherein the defoamer is selected from the group consisting of glycerides, waxes, powdered silica, ethylene oxide/propylene oxide block copolymers, silicone based defoamer and mixtures thereof.

19. Fluid according to one or more of claims 1 - 18, wherein the lubricant is selected from the group consisting of homopolymers of propylene oxide, copolymers of propylene oxide with ethylene oxide and/or butylene oxide, mono C₁ to C₄ alkyl substituted homopolymers of propylene oxide, mono C₁ to C₄ alkyl substituted copolymers of propylene oxide with ethylene oxide and/or butylene oxide, triglycerides, castor oil, ricinoleic acid, and ethoxylates of castor oil or ricinoleic acid, and mixtures thereof.

20. Fluid according to one or more of claims 1 - 19, comprising 0.1 to 3 wt.-% of an amine within the component (D), weight-% being relative to the fluid weight.

21. Fluid according to one or more of claims 1 - 20, wherein the fluid's content in esters between boric acid and glycol or alkyl polyglycol compounds is less than 3 wt.-%, preferably less than 1 wt.-%, more preferably 0.1 wt.-%, the fluid being most preferably essentially free of such boric acid ester.

22. Fluid according to one or more of claims 1 - 21, the fluid having a kinematic viscosity of less than 900 centistokes, preferably less than 750 centistokes at -40°C, on an dry equilibrium reflux boiling point (ERBP) of at least 250°C and a wet equilibrium reflux boiling point (WERBP) of at least 165°C, both ERBP and WERBP to be determined according to Federal Motor Vehicle Safety Standards (FMVSS) No 116.

23. Fluid according to one or more of claims 1 - 21, wherein R₅ is a C₁- to C₄-alkyl group.

24. Fluid according to one or more of claims 1 - 23, wherein component A) comprises a compound according to formula (Ia) wherein d is a number from 1 to 6, in an amount of up to 30 wt.-% relative to the total weight of all compounds according to formula (I).

25. Use of a fluid according to one or more of claims 1 - 24 as brake fluid.

26. Method of operating a vehicular brake, the method comprising transmitting hydraulic pressure by a fluid according to one or more of claims 1 - 24.

## Patentansprüche

1. Funktionsfluid umfassend
(A) von 8 bis 80 Gew.-%, bezogen auf das Gesamtgewicht der Zusammensetzung, an einem oder mehreren Orthoestern gemäß Formel (I) wobei
R1, R2, R3 unabhängig ausgewählt sind aus H und C₁- bis C₈-Alkylgruppen,
R4 H oder C₁- bis C₈-Alkyl bedeutet,
a, b, c unabhängig Zahlen von 0 bis 6 sind,
mit der Maßgabe, dass a+b+c wenigstens 1 beträgt,
(B) von 10 bis 87 Gew.-%, bezogen auf das Gesamtgewicht der Zusammensetzung, an einem oder mehreren Alkoxyglycolen gemäß Formel (II)
R₅-O- ( CH₂-CH₂-O)ₘ-H (II)
wobei
R₅ ein C₁- bis C₈-Alkylrest ist,
m eine Zahl von 2 bis 6 ist,
(C) von 0 bis 20 Gew.-% an wenigstens einer Verbindung gemäß Formel (III)
H-O- (CH₂-CH₂-O)ₖ-H (III)
wobei k eine Zahl von 2 oder größer ist, mit der Maßgabe, dass bei wenigstens 80 Gew.-% aller Verbindungen gemäß Formel (III) k 2 oder 3 ist,
(D) wenigstens einen Zusatzstoff ausgewählt aus der Gruppe bestehend aus Korrosionshemmer, Alkalinitätsmitteln, Alterungsschutzmitteln, Entschäumern und Schmiermitteln,
wobei das Fluid höchstens 3 Gew.-% an einem Ester zwischen Borsäure und einer Glycol- oder Polyglycolverbindung umfasst und
mit der Maßgabe, dass die kombinierte Menge von Komponente (A) und Komponente (B) eine Summe von wenigstens 70 % des Gesamtgewichts des Fluids bildet.

2. Fluid gemäß Anspruch 1, wobei die Komponenten (A) bis (D) eine Summe von 100 Gew.-% bilden.

3. Fluid gemäß Anspruch 1 oder 2, wobei R1, R2, R3 unabhängig ausgewählt sind aus H und C₁- bis C₄-Alkylgruppen.

4. Fluid gemäß einem oder mehreren der Ansprüche 1-3, wobei R1, R2, R3 unabhängig ausgewählt sind aus Methyl- und Butylgruppen.

5. Fluid gemäß einem oder mehreren der Ansprüche 1-4, wobei R4 H oder C₁- bis C₄-Alkyl ist.

6. Fluid gemäß einem oder mehreren der Ansprüche 1-5, wobei R4 H oder Methyl ist.

7. Fluid gemäß einem oder mehreren der Ansprüche 1-6, wobei a+b+c wenigstens 3, bevorzugter wenigstens 6, beträgt.

8. Fluid gemäß einem oder mehreren der Ansprüche 1-6, wobei a, b, c unabhängig 3 oder 4 sind.

9. Fluid gemäß einem oder mehreren der Ansprüche 1-8, wobei die Komponente (A) ein Gemisch von wenigstens zwei Verbindungen gemäß Formel (I) ist, die sich in einem von R1, R2, R3 oder in einem von a, b, c unterscheiden.

10. Fluid gemäß einem oder mehreren der Ansprüche 1-9, wobei bei wenigstens 60 Gew.-% aller Verbindungen gemäß Formel (II) m 3 oder 4 ist.

11. Fluid gemäß einem oder mehreren der Ansprüche 1-9, wobei Komponente (C) in einer Menge von 4 bis 18 Gew.-% vorhanden ist.

12. Fluid gemäß einem oder mehreren der Ansprüche 1-11, wobei bei höchstens 10 Gew.-% aller Verbindungen gemäß Formel (II) m 5 oder höher ist.

13. Fluid gemäß einem oder mehreren der Ansprüche 1-12, wobei das Fluid höchstens 10 Gew.-% an Verbindungen gemäß Formel (III) enthält, wobei k 4 oder größer ist, wobei die Gew.-% auf das Gesamtgewicht der Komponente C bezogen sind.

14. Fluid gemäß einem oder mehreren der Ansprüche 1-13, wobei Komponente (D) in einer Menge von 0,2 bis 6 Gew.-%, vorzugsweise 0,4 bis 4,5 Gew.-%, vorhanden ist.

15. Fluid gemäß einem oder mehreren der Ansprüche 1-14, wobei der Korrosionshemmer ausgewählt ist aus der Gruppe bestehend aus C₈- bis C₂₂-Fettsäuren, Estern von phosphoriger oder Phosphorsäure mit C₁- bis C₁₈-aliphatischen Alkoholen, Phosphiten mit wenigstens einem C₁- bis C₁₂-Kohlenwasserstoffrest, heterocyclischen organischen Verbindungen mit wenigstens einem Stickstoffatom als Heteroatom, und Gemischen davon.

16. Fluid gemäß einem oder mehreren der Ansprüche 1-15, wobei das Alkalinitätsmittel ausgewählt ist aus der Gruppe bestehend aus Alkyl- oder Cycloalkylaminen, Alkanolaminen, Alkylaminethoxylaten und deren Gemischen.

17. Fluid gemäß einem oder mehreren der Ansprüche 1-16, wobei das Alterungsschutzmittel ausgewählt ist aus der Gruppe bestehend aus substituierten Phenolen, sterisch gehinderten Aminen und Gemischen davon.

18. Fluid gemäß einem oder mehreren der Ansprüche 1-17, wobei der Entschäumer ausgewählt ist aus der Gruppe bestehend aus Glyceriden, Wachsen, pulverförmigem Siliciumdioxid, Ethylenoxid/Propylenoxid-Blockcopolymeren, Entschäumer auf Siliconbasis und Gemischen davon.

19. Fluid gemäß einem oder mehreren der Ansprüche 1-18, wobei das Schmiermittel ausgewählt ist aus der Gruppe bestehend aus Homopolymeren von Propylenoxid, Copolymeren von Propylenoxid mit Ethylenoxid und/oder Butylenoxid, mono-C₁-bis-C₄-alkylsubstituierten Homopolymeren von Propylenoxid, mono-C₁-bis-C₄-alkylsubstituierten Copolymeren von Propylenoxid mit Ethylenoxid und/oder Butylenoxid, Triglyceriden, Rizinusöl, Ricinolsäure und Ethoxylaten von Rizinusöl oder Ricinolsäure, und Gemischen davon.

20. Fluid gemäß einem oder mehreren der Ansprüche 1-19, umfassend 0,1 bis 3 Gew.-% an einem Amin in der Komponente (D), wobei die Gew.-% auf das Fluidgewicht bezogen sind.

21. Fluid gemäß einem oder mehreren der Ansprüche 1-20, wobei der Gehalt des Fluids an Estern zwischen Borsäure und Glycol- oder Alkylpolyglycolverbindungen weniger als 3 Gew.-%, vorzugsweise weniger als 1 Gew.-%, bevorzugter 0,1 Gew.-%, beträgt, wobei das Fluid höchst bevorzugt im Wesentlichen frei von derartigem Borsäureester ist.

22. Fluid gemäß einem oder mehreren der Ansprüche 1-21, wobei das Fluid eine kinematische Viskosität von weniger als 900 Centistokes, vorzugsweise weniger als 750 Centistokes, bei -40 °C an einem Trockengleichgewichtssiedepunkt unter Rückfluss (ERBP) von wenigstens 250 °C und einem Nassgleichgewichtssiedepunkt unter Rückfluss (WERBP) von wenigstens 165 °C aufweist, wobei sowohl ERBP als auch WERBP nach Federal Motor Vehicle Safety Standards (FMVSS) Nr. 116 zu bestimmen sind.

23. Fluid gemäß einem oder mehreren der Ansprüche 1-21, wobei R₅ eine C₁- bis C₄-Alkylgruppe ist.

24. Fluid gemäß einem oder mehreren der Ansprüche 1-23, wobei Komponente A) eine Verbindung gemäß Formel (Ia), wobei d eine Zahl von 1 bis 6 ist, in einer Menge bis 30 Gew.-% bezogen auf das Gesamtgewicht aller Verbindungen gemäß Formel (I) umfasst.

25. Verwendung eines Fluids gemäß einem oder mehreren der Ansprüche 1-24 als Bremsfluid.

26. Verfahren zum Betreiben einer Fahrzeugbremse, wobei das Verfahren Übertragen von hydraulischem Druck durch ein Fluid gemäß einem oder mehreren der Ansprüche 1-24 umfasst.

## Revendications

1. Fluide fonctionnel, comprenant
(A) de 8 à 80 % en poids, sur la base de la composition totale, d'un ou plusieurs orthoesters selon la formule (I)
R1, R2, R3 étant indépendamment choisis parmi H ou des groupes alkyle en C₁₋₈,
R4 signifiant H ou alkyle en C₁₋₈,
a, b, c étant indépendamment des nombres de 0 à 6,
à la condition que a + b + c soit au moins 1,
(B) de 10 à 87 % en poids, sur la base de la composition totale, d'un ou plusieurs alcoxy glycols selon la formule (II)
R₅ - O - (CH₂ - CH₂ - O)ₘ - H (II)
R₅ étant un radical alkyle en C₁₋₈,
m étant un nombre de 2 à 6,
(C) de 0 à 20 % en poids d'au moins un composé selon la formule (III)
H -O- (CH₂ - CH₂ - O)ₖ - H (III)
k étant un nombre de 2 ou plus, à la condition que dans au moins 80 % en poids de tous les composés selon la formule (III), k soit 2 ou 3,
(D) au moins un additif, choisi dans le groupe constitué par un inhibiteur de corrosion, des agents d'alcalinité, des agents de protection contre le vieillissement, des antimousses et des lubrifiants,
le fluide comprenant au plus 3 % en poids d'un ester entre l'acide borique et un composé de glycol ou de polyglycol, et
à la condition que la quantité combinée de composant (A) et de composant (B) totalise jusqu'à au moins 70 % du poids du fluide total.

2. Fluide selon la revendication 1, les composants (A) à (D) totalisant jusqu'à 100 en poids.

3. Fluide selon la revendication 1 ou 2, R1, R2, R3 étant indépendamment choisis parmi H ou des groupes alkyle en C₁₋₄.

4. Fluide selon l'une ou plusieurs des revendications 1 à 3, R1, R2, R3 étant indépendamment choisis parmi des groupes méthyle et butyle.

5. Fluide selon l'une ou plusieurs des revendications 1 à 4, R4 étant H ou alkyle en C₁₋₄.

6. Fluide selon l'une ou plusieurs des revendications 1 à 5, R4 étant H ou méthyle.

7. Fluide selon l'une ou plusieurs des revendications 1 à 6, a + b + c étant au moins 3, plus préférablement au moins 6.

8. Fluide selon l'une ou plusieurs des revendications 1 à 6, a, b, c étant indépendamment 3 ou 4.

9. Fluide selon l'une ou plusieurs des revendications 1 à 8, le composant (A) étant un mélange d'au moins deux composés selon la formule (I) qui diffèrent dans l'un parmi R1, R2, R3 ou dans l'un parmi a, b, c.

10. Fluide selon l'une ou plusieurs des revendications 1 à 9, dans au moins 60 % en poids de tous les composés selon la formule (II), m étant 3 ou 4.

11. Fluide selon l'une ou plusieurs des revendications 1 à 9, le composant (C) étant présent en une quantité de 4 à 18 % en poids.

12. Fluide selon l'une ou plusieurs des revendications 1 à 11, dans au plus 10 % en poids de tous les composés selon la formule (II), m étant 5 ou plus.

13. Fluide selon l'une ou plusieurs des revendications 1 à 12, le fluide contenant au plus 10 % en poids de composés selon la formule (III) dans laquelle k est 4 ou plus, le % en poids étant par rapport au poids total du composant C.

14. Fluide selon l'une ou plusieurs des revendications 1 à 13, le composant (D) étant présent en une quantité de 0,2 à 6 % en poids, préférablement 0,4 à 4,5 % en poids.

15. Fluide selon l'une ou plusieurs des revendications 1 à 14, l'inhibiteur de corrosion étant choisi dans le groupe constitué par des acides gras en C₈₋₂₂, des esters de phosphore ou d'acide phosphorique avec des alcools aliphatiques en C₁₋₁₈, des phosphites ayant au moins un radical hydrocarboné en C₁₋₁₂ ; des composés organiques hétérocycliques ayant au moins un atome de nitrogène en tant qu'hétéroatome, et des mélanges correspondants.

16. Fluide selon l'une ou plusieurs des revendications 1 à 15, l'agent d'alcalinité étant choisi dans le groupe constitué par des alkylamines ou cycloalkylamines, des alcanolamines, des éthoxylates d'alkylamine et leurs mélanges.

17. Fluide selon l'une ou plusieurs des revendications 1 à 16, l'agent de protection contre le vieillissement étant choisi dans le groupe constitué par des phénols substitués, des amines stériquement encombrées et des mélanges correspondants.

18. Fluide selon l'une ou plusieurs des revendications 1 à 17, l'antimousse étant choisi dans le groupe constitué par des glycérides, des cires, une silice en poudre, des copolymères à blocs d'oxyde d'éthylène/oxyde de propylène, un antimousse à base de silicone et des mélanges correspondants.

19. Fluide selon l'une ou plusieurs des revendications 1 à 18, le lubrifiant étant choisi dans le groupe constitué par des homopolymères d'oxyde de propylène, des copolymères d'oxyde de propylène avec l'oxyde d'éthylène et/ou l'oxyde de butylène, des homopolymères monosubstitués par alkyle en C₁₋₄ d'oxyde de propylène, des copolymères monosubstitués par alkyle en C₁₋₄ d'oxyde de propylène avec l'oxyde d'éthylène et/ou l'oxyde de butylène, des triglycérides, l'huile de ricin, l'acide ricinoléique, et des éthoxylates d'huile de ricin ou d'acide ricinoléique, et des mélanges correspondants.

20. Fluide selon l'une ou plusieurs des revendications 1 à 19, comprenant 0,1 à 3 % en poids d'une amine dans le composant (D), le % en poids étant par rapport au poids du fluide.

21. Fluide selon l'une ou plusieurs des revendications 1 à 20, la teneur en fluide dans des esters entre l'acide borique et des composés de glycol ou d'alkyl polyglycol étant inférieure à 3 % en poids, préférablement inférieure à 1 % en poids, plus préférablement 0,1 % en poids, le fluide étant le plus préférablement essentiellement exempt d'un tel ester d'acide borique.

22. Fluide selon l'une ou plusieurs des revendications 1 à 21, le fluide ayant une viscosité cinématique inférieure à 900 centistokes, préférablement inférieure à 750 centistokes à une température de - 40 °C, sur un point d'ébullition au reflux à l'équilibre sec (ERBP) d'au moins 250 °C et un point d'ébullition au reflux à l'équilibre humide (WERBP) d'au moins 165 °C, à la fois ERBP et WERBP devant être déterminés selon les normes fédérales de sécurité de véhicules à moteur (FMVSS) n° 116.

23. Fluide selon l'une ou plusieurs des revendications 1 à 21, R₅ étant un groupe alkyle en C₁₋₄.

24. Fluide selon l'une ou plusieurs des revendications 1 à 23, le composant A) comprenant un composé selon la formule (Ia) d étant un nombre de 1 à 6, en une quantité allant jusqu'à 30 % en poids par rapport au poids total de tous les composés selon la formule (I).

25. Utilisation d'un fluide selon l'une ou plusieurs des revendications 1 à 24 comme fluide de frein.

26. Procédé d'exploitation d'un frein de véhicule, le procédé comprenant la transmission d'une pression hydraulique par un fluide selon l'une ou plusieurs des revendications 1 à 24.
